

# United States Patent

Hiller

[15] 3,649,289

[45] Mar. 14, 1972

[54] **PHOTOGRAPHIC MATERIALS**

[72] Inventor: **Gary L. Hiller**, Rochester, N.Y.

[73] Assignee: **Eastman Kodak Company**, Rochester, N.Y.

[22] Filed: **Oct. 21, 1968**

[21] Appl. No.: **769,393**

[52] U.S. Cl. .... **96/123, 96/107, 96/126**

[51] Int. Cl. .... **G03c 1/10**

[58] Field of Search..... **96/104, 127, 126, 107, 95, 96/94**

|           |         |                    |        |
|-----------|---------|--------------------|--------|
| 3,041,170 | 6/1962  | Haist et al.....   | 96/95  |
| 3,155,518 | 11/1964 | Blake.....         | 96/95  |
| 3,155,519 | 11/1964 | Blake.....         | 96/95  |
| 3,177,210 | 4/1965  | Rosenoff.....      | 96/106 |
| 3,189,454 | 6/1965  | Luckey et al. .... | 96/95  |
| 3,305,363 | 2/1967  | Beavers et al..... | 96/95  |

FOREIGN PATENTS OR APPLICATIONS

|           |         |                     |        |
|-----------|---------|---------------------|--------|
| 742,112   | 12/1955 | Great Britain ..... | 96/106 |
| 1,066,070 | 4/1967  | Great Britain ..... | 96/106 |

Primary Examiner—William D. Martin

Assistant Examiner—William R. Trenor

Attorney—W. H. J. Kline, J. R. Frederick and O. H. Webster

[56] **References Cited**

UNITED STATES PATENTS

|           |         |                   |        |
|-----------|---------|-------------------|--------|
| 3,442,649 | 5/1969  | Rasch et al. .... | 96/94  |
| 2,503,776 | 4/1950  | Sprague .....     | 96/106 |
| 2,947,630 | 8/1960  | Jones.....        | 96/104 |
| 2,961,318 | 11/1960 | Jones.....        | 96/104 |

[57] **ABSTRACT**

Photographic silver halide emulsions are spectrally sensitized with the combination of complex merocyanine dye, sulfonated polynuclear aromatic compound and reducing agent.

9 Claims, No Drawings

## PHOTOGRAPHIC MATERIALS

This invention relates to novel photographic materials, and more particularly to spectrally sensitized photographic silver halide emulsions.

The spectral sensitization of photographic silver halide emulsions with supersensitizing combinations comprising various methine dyes with sulfonated organic compounds has been described previously, such as in U.S. Pat. Nos. 2,875,058; 2,933,390; 2,945,762; 2,947,630, and 2,961,318. When photographic silver halide emulsions are spectrally sensitized with complex merocyanine dyes, an undesirable reduction in the blue sensitivity of the emulsion results. While the addition of sulfonated polynuclear organic compounds increases the blue speed of emulsions containing complex merocyanine dyes, it would be highly desirable to provide emulsions containing complex merocyanine dyes which have even higher inherent blue speeds than are obtained with a combination of sulfonated polynuclear organic compound and complex merocyanine dye.

One object of this invention is to provide novel spectral sensitizing combinations for photographic silver halide emulsions.

Another object of this invention is to provide photographic silver halide emulsions containing complex merocyanine dyes which have good speed when exposed to blue radiation.

Other objects of this invention will be apparent from the disclosure herein and the appended claims.

In accordance with this invention, photographic silver halide emulsions are spectrally sensitized with the combination of complex merocyanine dye, sulfonated polynuclear organic supersensitizer and, a sufficient amount of a silver halide reducing agent to effectively increase the blue speed of the emulsion. It has been found that utilization of sulfonated polynuclear organic supersensitizer in combination with reducing agent materially increases the response to blue radiation (about 350 to 500 nm.) of silver halide emulsions spectrally sensitized with complex merocyanine dyes. This result is particularly surprising in view of the fact that the use of reducing agent in photographic silver halide emulsions containing sulfonated organic supersensitizer and various classes of methine dyes fails to result in any substantial increase in the blue speed of the emulsion. It could not have been foreseen that the combination of reducing agent and sulfonated polynuclear supersensitizer would in some manner coact to substantially enhance the blue speed of emulsions spectrally sensitized with complex merocyanine dye.

As used herein and in the appended claims, the term "complex merocyanine" dye refers to methine dyes having three five- to six-membered nitrogen containing heterocyclic nuclei joined at carbon atoms thereof by a double bond or a methine (preferably dimethine) linkage, one terminal nucleus being a basic heterocyclic nucleus of the type used in cyanine dyes, and the other two nuclei being acidic ketomethylene heterocyclic nuclei of the type used in merocyanine dyes, said dye having an amidic chromophoric system. See "The Theory of the Photographic Process" by Mees and James, third edition, page 201 (1966), The MacMillan Company, New York.

The complex merocyanine dyes that are preferred in practicing this invention are those represented by the following formula:



wherein  $n$  represents a positive integer of from 1 to 2;  $m$  and  $p$  each represents a positive integer of from 1 to 3;  $L$  represents a methine linkage, e.g.,  $=CH-$ ,  $=C(CH_3)_2-$ ,  $=C(C_6H_5)_2-$ , etc.;  $A$  represents an atom of sulfur, or the group  $=N-R_3$  wherein  $R_3$  represents an alkyl group containing from one to four carbon atoms), e.g., methyl, ethyl, propyl, isopropyl, butyl, etc.; or an aryl group, e.g., phenyl, tolyl, naphthyl, methoxyphenyl, chlorophenyl, etc.;  $R_1$  represents an alkyl group, including substituted alkyl, (preferably a lower alkyl containing from one to four carbon atoms), e.g., methyl, ethyl, propyl,

isopropyl, butyl, hexyl, cyclohexyl, decyl, dodecyl, etc., and substituted alkyl groups (preferably a substituted lower alkyl) containing from one to four carbon atoms), such as a hydroxalkyl group, e.g.,  $\beta$ -hydroxy-ethyl,  $\omega$ -hydroxybutyl, etc., an alkoxalkyl group, e.g.,  $\beta$ -methoxyethyl,  $\omega$ -butoxybutyl, etc., a carboxyalkyl group, e.g.,  $\beta$ -carboxyethyl,  $\omega$ -carboxybutyl, etc.; a sulfoalkyl group, e.g.,  $\beta$ -sulfoethyl,  $\omega$ -sulfobutyl, etc., a sulfatoalkyl group, e.g.,  $\beta$ -sulfatoethyl,  $\omega$ -sulfobutyl, etc., an acyloxyalkyl group, e.g.,  $\beta$ -acetoxymethyl,  $\nu$ -acetoxypropyl,  $\omega$ -butyryloxybutyl, etc., an alkoxy carbonylalkyl group, e.g.,  $\beta$ -methoxycarbonylethyl,  $\omega$ -ethoxycarbonylbutyl, etc., or an aralkyl group, e.g., benzyl, phenethyl, etc., or, an aryl group, e.g., phenyl, tolyl, naphthyl, methoxyphenyl, chlorophenyl, etc.;  $R_2$  represents an alkyl group containing from one to four carbon atoms, e.g., methyl, butyl, etc., or an aryl group, e.g., phenyl, tolyl, chlorophenyl, methoxyphenyl, naphthyl, etc.;  $Z$  represents the nonmetallic atoms necessary to complete a five- to six-membered heterocyclic nucleus, which nucleus may contain a second hetero atom such as oxygen, sulfur, selenium or nitrogen, such as the following nuclei: a thiazole nucleus, e.g., thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 5-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole, naphtho[2,1-d]thiazole, naphtho[1,2-d]thiazole, 5-methoxynaphtho[2,3-d]thiazole, 5-ethoxynaphtho[2,3-d]thiazole, 8-methoxynaphtho[2,3-d]thiazole, 7-methoxynaphtho[2,3-d]thiazole, 4'-methoxythianaphtho-7',6',4,5-thiazole, etc.; an oxazole nucleus, e.g., 4-methyloxazole, 5-methyloxazole, 4-phenyloxazole, 4,5-diphenyloxazole, 4-ethyloxazole, 4,5-dimethyloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole, naphtho[2,1-d]oxazole, naphtho[1,2-d]oxazole, etc.; a selenazole nucleus, e.g., 4-methylselenazole, 4-phenylselenazole, 5-chlorobenzoselenazole, 5-methoxybenzoselenazole, 5-hydroxybenzoselenazole, tetrahydrobenzoselenazole, naphtho[2,1-d]selenazole, naphtho[1,2-d]selenazole, etc.; a thiazoline nucleus, e.g., thiazoline, 4-methylthiazoline, etc.; a pyridine nucleus, e.g., 2-pyridine, 5-methyl-2-pyridine, 4-pyridine, 3-methyl-4-pyridine, etc.; a quinoline nucleus, e.g., 2-quinoline, 3-methyl-2-quinoline, 5-ethyl-2-quinoline, 6-chloro-2-quinoline, 8-chloro-2-quinoline, 6-methoxy-2-quinoline, 8-ethoxy-2-quinoline, 8-hydroxy-2-quinoline, 4-quinoline, 6-methoxy-4-quinoline, 7-methyl-4-quinoline, 8-chloro-4-quinoline, 1-isoquinoline, 3,4-dihydro-1-isoquinoline, 3-

isoquinoline, etc.; a 3,3-dialkylindolenine nucleus, e.g., 3,3-dimethylindolenine, 3,3,5-trimethylindolenine, etc.; and, an imidazole nucleus, e.g., imidazole, 1-alkylimidazole, 1-alkyl-4-phenylimidazole, 1-alkyl-4,5-dimethylimidazole, benzimidazole, 1-alkylbenzimidazole, 1-aryl-5,6-dichlorobenzimidazole, 1-alkyl-1H-naphth[1,2-d]imidazole, 1-aryl-3H-naphth[1,2-d]imidazole, 1-alkyl-5-methoxy-1H-naphth[1,2-d]imidazole, etc.; and Q represents atoms necessary to complete a five- or six-membered nucleus, typically containing a hetero atom selected from nitrogen and sulfur.

such as a 2-pyrazolin-5-one nucleus, e.g., 3-methyl-1-phenyl-2-pyrazolin-5-one, 1-phenyl-2-pyrazolin-5-one, 1-(2-benzothiazolyl)-3-methyl-2-pyrazolin-5-one, etc.; a 2,4,6-triketohexahydropyrimidine nucleus, e.g., 2-thiobarbituric acid as well as its 1-alkyl (e.g., 1-methyl, 1-ethyl, 1-propyl, 1-heptyl, etc.) or 1,3-dialkyl (e.g., 1,3-dimethyl, 1,3-diethyl, 1,3-dipropyl, 1,3-diisopropyl, 1,3-dicyclohexyl, 1,3-di( $\beta$ -methoxyethyl), etc.; or 1,3-diaryl (e.g., 1,3-diphenyl, 1,3-di(p-chlorophenyl), 1,3-di(p-ethoxycarbonylphenyl), etc.); or 1-aryl (e.g., 1-phenyl, 1-p-chlorophenyl, 1-p-ethoxycarbonylphenyl, etc.) or 1-alkyl-3-aryl (e.g., 1-ethyl-3-phenyl, 1-n-heptyl-3-phenyl, etc.) derivatives; and a rhodanine nucleus (i.e., 2-thio-2,4-thiazolidinedione series), such as rhodanine, 3-alkylrhodanines, e.g., 3-ethylrhodanine, 3-allylrhodanine, etc., 3-carboxyalkylrhodanines, e.g., 3-(2-carboxyethyl)rhodanine, 31(4-carboxybutyl)rhodanine, etc. 3-sulfoalkylrhodanines, e.g., 3-(2-sulfoethyl)rhodanine, 3-(3-sulfopropyl)rhodanine, 3-(4-sulfonylbutyl)rhodanine, etc., or 3-arylrhodanines, e.g., 3-phenylrhodanine, etc., etc.

Included among the complex merocyanine dyes defined by Formula I above are the following typical dye compounds.

TABLE A

| Dye No. | Dye compound                                                                                                                                               |
|---------|------------------------------------------------------------------------------------------------------------------------------------------------------------|
| I       | 1-Ethyl-4-[(3-ethyl-2-benzothiazolinylidene)ethylidene]-2-[(3-ethyl-4-oxo-2-thioxo-5-thiazolidinylidene)ethylidene]-3-phenyl-5-imidazolidinone             |
| II      | 1,3-Diethyl-5-[(1-ethylnaphtho[1,2-d]thiazolin-2-ylidene)ethylidene]-2-[(3-ethyl-4-oxo-2-thioxo-5-thiazolidinylidene)ethylidene]-4-imidazolidinone         |
| III     | 3-Ethyl-2-[(1-ethylhexahydro-4,6-dioxo-2-thioxo-5-pyrimidinylidene)ethylidene]-1-phenyl-5-[(1,3,5-trimethyl-2-indolinylidene)ethylidene]-4-imidazolidinone |
| IV      | 1,3-Diethyl-5-[(3-ethyl-2-benzothiazolinylidene)-ethylidene]-2-[(3-methyl-5-oxo-1-phenyl-2-pyrazolin-4-ylidene)ethylidene]-4-imidazolidinone               |
| V       | 3-Ethyl-5-[(1-ethyl-2-(1H)- $\beta$ -naphthoselenazolylidene)-isopropylidene]-2-(3-ethyl-4-oxo-2-thioxo-5-thiazolidinylidene)-4-thiazolidinone             |
| VI      | 3-Ethyl-5-[(3-ethyl-2-benzoxazolinylidene)ethylidene]-2-[(3-ethyl-4-oxo-2-thioxo-5-thiazolidinylidene)-ethylidene]-4-thiazolidinone                        |
| VII     | 3-Ethyl-5-[(1-ethylnaphtho[1,2-d]thiazolin-2-ylidene)ethylidene]-2-[(3-ethyl-4-oxo-2-thioxo-5-thiazolidinylidene)ethylidene]-em-1-phenyl-4-imidazolidinone |

The complex merocyanine dyes represented by above Dye No. V have previously been described in the prior art in references such as Fry et al. U.S. Pat. No. 2,388,913, issued Nov. 13, 1945; Brooker, U.S. Pat. No. 2,454,629, issued Nov. 23, 1948; Aubert et al., U.S. Pat. No. 2,656,351, issued Oct. 20, 1953; etc. Dyes represented by Dye Nos. I, II, III, IV, VI and VII can be conveniently prepared by the general process described in copending application Jenkins, Ser. No. 657,082, filed July 31, 1967, entitled "Synthesis of Trinuclear Dyes." Thus, the above-mentioned dyes are prepared by condensing a compound of the formula:



with a compound of the formula:

III.



wherein  $n$ ,  $m$ ,  $p$ ,  $L$ ,  $A$ ,  $R_1$ ,  $R_2$ ,  $Z$  and  $Q$  are as previously defined, and  $X$  represents an acid anion, e.g., chloride, bromide, iodide, sulfamate, perchlorate, p-toluenesulfonate, methyl sulfate, etc., in a suitable solvent, in approximately equimolar proportions and in the presence of a basic condensing agent such as triethylamine, the dyes being separated and purified by one or more recrystallizations from an appropriate solvent.

The following example illustrates the above process with the preparation of above Dye No. II: 1,3-Diethyl-5-[(1-ethyl-naphtho[1,2-d]thiazolin-2-ylidene)-ethylidene]-2-[(3-ethyl-4-oxo-2-thioxo-5-thiazolidinylidene)ethylidene]-4-imidazolidinone

20



30 1,3-Diethyl-5-[(1-ethylnaphtho[1,2-d]thiazolin-2-ylidene)ethylidene]-2-methyl-4-oxo-2-imidazolinium iodide (1 mol., 1.30 g.), 5-acetanilidomethylene-3-ethylrhodanine (1 mol., 0.80 g.), acetic anhydride (200 percent excess, 0.50 g.) and triethylamine (1 mol.+200 percent, 0.75 g.) was dissolved in pyridine (10 ml.) and the solution was heated under reflux for twenty minutes. The hot reaction mixture was transferred to a beaker containing acetic anhydride (2.0 ml.). The warm solution was treated first with *N,N*-diethylethylenediamine (2.0 ml.) and then diluted with methanol (125 ml.). The solution was chilled overnight and the crude dye was collected by filtration, washed with methanol and dried. The crude dye was recrystallized by dissolving in hot pyridine containing acetic anhydride. The resulting solution was first treated with *N,N*-diethylethylenediamine and then diluted with methanol. The solution was chilled and the dye was collected by filtration, washed with methanol and dried. After a final recrystallization from pyridine and methanol, the yield of pure dye was 0.45 g. (32 percent), m.p. 253.0°-255.0°C. dec.

The sulfonated organic supersensitizers useful in practicing my invention comprise polynuclear aromatic compounds containing at least one sulfo group. The term "polynuclear aromatic" as used herein is intended to mean two or more benzene rings fused together (for example, as in naphthalene, pyrene, etc.) or at least two benzene rings of aromatic rings directly joined together (for example, as in diphenyl, terphenyl, quaterphenyl, etc.) or through an aliphatic linkage. Such sulfonated derivatives can conveniently be represented by the following general formula:

IV.  $\text{D-SO}_3\text{M}$ 

60 wherein  $\text{D}$  represents a polynuclear aromatic group as defined above and  $\text{M}$  represents a hydrogen atom or a water-soluble cation salt group (e.g., sodium, potassium, ammonium, triethylammonium, triethanolammonium, pyradinium, etc.). Among the most useful of the sulfonated derivatives embraced by Formula IV above are the compounds represented by the following general formula:

V.



70

wherein  $B_1$  represents a 1,3,5-triazin-6-ylamino group,  $B_2$  represents an aromatic group (i.e., benzene or substituted benzene) and  $M$  has the values given above.

Typical of the sulfonated derivatives of Formula V above, wherein  $B_1$  represents a 1,3,5-triazin-6-ylamino group (i.e., a 1,3,5-triazin-2-ylamino group) are the compounds selected from those represented by the following general formula:



wherein M has the values given above and R<sub>4</sub>, R<sub>5</sub>, R<sub>6</sub>, R<sub>7</sub> each represents a hydrogen atom or a substituent group, such as hydroxyl, aryloxyl (e.g., phenoxy, o-toloxyl, p-sulfophenoxy, etc.), alkoxy (e.g., methoxyl, ethoxyl, etc.), a halogen atom (e.g., chlorine, bromine, etc.), a heterocyclic radical (e.g., morpholinyl, piperidyl, etc.), an alkylthio group (e.g., methylthio, ethylthio, etc.), an arylthio group (e.g., phenylthio, tolylthio, etc.), a heterocyclythio group (e.g., benzothiazylthio, etc.) an amino group, an alkylamino group (e.g., methylamino, ethylamino, propylamino, dimethylamino, diethylamino, dodecylamino, cyclohexylamino,  $\beta$ -hydroxyethylamino, di- $\beta$ -hydroxyethylamino,  $\beta$ -sulfoethylamino, etc.), an arylamino group (e.g., anilino, o-, m- and p-anisylamino, o-, m- and p-chloroanilino, o-, m- and p-toluidino, o-, m-, and p-carboxyanilino, hydroxyanilino, sulfonaphthylamino, o-, m- and p-aminoanilino, p-acetamidoanilino, etc.), etc.

Compounds of Formula Va wherein  $R_4$ ,  $R_5$ ,  $R_6$  and/or  $R_7$ , each represents a heterocyclamino group (e.g., 2-benzothiazoleamino, 2-pyridylamino, etc.) can also be used in practicing my invention.



Another group of sulfonated derivatives which are useful in practicing my invention are those represented by the following general formula:



wherein  $R_8$  is an acylamido group (e.g., acetamido, sulfonybenzamido, 4-methoxy-3-sulfonybenzamido, 2-ethoxybenzamido, 2,4-diethoxy, benzamido, p-tolylamido, 4-methyl-2-methoxybenzamido, 1-naphthoylamino, 2-naphthoylamino, 2,4-dimethoxybenzamido, 2-phenylbenzamido, 2-thienylbenzamido) or a sulfo group,  $R_9$  represents an acylamido group (e.g., as defined by  $R_8$  above), or a sulfoaryl group (e.g., sulfophenyl, p'-sulfodiphenyl, etc.) and  $R_{10}$  represents a hydrogen atom or a sulfo group, said compound containing at least one sulfo group.

Compounds of Formula Va which can advantageously be employed in practicing my invention have been described in one or more of the following representative patents: U.S.:

|           |               |
|-----------|---------------|
| 2,171,427 | Aug. 29, 1939 |
| 2,473,475 | June 14, 1949 |
| 2,595,030 | Apr. 29, 1952 |
| 2,660,578 | Nov. 24, 1953 |
| 2,945,762 | July 19, 1960 |

### British:

|         |               |
|---------|---------------|
| 595,065 | Nov. 26, 1947 |
| 623,849 | May 24, 1949  |
| 624,051 | May 26, 1949  |
| 624,052 | May 26, 1949  |
| 678,291 | Sept. 3, 1952 |
| 681,642 | Oct. 29, 1952 |
| 705,406 | Mar. 10, 1954 |

The products of Formula *Va* have been previously employed in the textile field, and are sold under such tradenames as Leucophor B, Calcofluor White MR, Tinopal (SP, WR, BV277, 2B, GS, NG), Blancofor SC, Hiltamine (BSP, N, Sol. 6T6), and the like.

The dibenzothiophenedioxide compounds of Formula VI have, in general, been previously described in the prior art. See, for example, U.S. Pat. Nos. 2,573,652; 2,580,234; and 2,563,493. Further examples of the preparation of such compounds are given in J. E. Jones, J. Spence, and J. A. Van Allan, U.S. Pat. No. 2,937,089, issued May 17, 1960. Other examples of sulfonated derivatives embraced by Formula IV above which can advantageously be used in my invention can be prepared according to the methods described in application Ser. No. 575,160. Still other examples of compounds represented by Formula IV above which can be used in my invention have been previously described in B. H. Carroll, J. E. Jones, and J. Spence, U.S. Pat. 2,950,196, issued Aug. 23, 1960. (See, in particular, the compounds of Formulas II, III and IV of that patent).

Compounds selected from those of Formula V above wherein B<sub>1</sub> represents a 2-benzotriazolyl group can be prepared according to methods previously described in the prior art. See, for example, U.S. Pat. to Zweidler et al. No. 2,713,057, dated July 12, 1955; Keller et al., U.S. Pat. No. 2,684,966, dated July 27, 1954; Zweidler et al., U.S. Pat. No. 2,784,197, dated Mar. 5, 1957; and Keller et al., U.S. Pat. No. 2,784,183, dated Mar. 5, 1957. A somewhat related group of compounds containing a 2-benzotriazolyl group which can be used in my invention have been previously described in U.S. Pat. No. 2,733,165. Such compounds are embraced by Formula IV above.

Typical sulfonated derivatives embraced by Formulas IV, V, Va and VI above are (chemical formulas are given for various types to aid in identification): 1. a sulfonated triazolostilbene, e.g., of the type shown in U.S. Pat. No. 2,713,057.



- 45 4,4'-di(4'', 6''-dihydroxy-2''-s-triazinylamino)stilbene-2,2'-disulfonic acid 3. 4,4'-bis[4-(3'-sulfoanilino)-6-amino-s-triazin-2-ylamino]-stilbene

4. Tinopal-WR, a sulfonated triazinyl stilbene

5. Tinopal-2B, a sulfonated triazinyl stilbene

50 6. A sulfonated triazinyl stilbene, e.g., of the type shown in U.S. Pat. No. 2,595,030, or British Pat. No. 595,065

7. 4,4'-bis[2-(4-sulfoanilino-2- $\beta$ -hydroxyethylamino)-1,3,5-triazin-6-ylamino]stilbene-2,2'-disulfonic acid

8. 4,4'-bis(2,4-dihydroxy-1,3,5-triazin-6-ylamino)dibenzyl-2,2'-disulfonic acid

55 9. 4,4'-bis(2- $\beta$ -hydroxyethylamino-4-anilino-1,3,5-triazin-6-ylamino)-1,4-distyrylbenzene-2,2'-disulfonic acid

10. 5-methoxy-2-(4-styryl-3-sulfo)phenyl-1,2,3-benzotriazole sodium salt

11. Calcofluor White-MR, a sulfonated triazinyl stilbene



70

3,7-bis(2-phenylbenzamido)-2,8-disulfodibenzothiophene-  
5,5-dioxide  
13. 3,7-bis(2-thienylamido)-2,8disulfodibenzothiophene diox-  
ide sodium salt  
14. 3-[4-(4-methoxy-3-sulfobenzamido)phenyl]-7-(4-  
methoxy-3-sulfobenzamido)dibenzothiophene dioxide sodium  
salt

15. chrysens-6-sulfonic acid sodium salt  
 16. pyrene-3-sulfonic acid sodium salt  
 17. Phenanthrene-3-sulfonic acid sodium salt  
 18. 2,3-dimethylnaphthalene-1-sulfonic acid sodium salt  
 19. 4-[-phenoxy-6-( $\beta$ -hydroxyethylamino)-s-triazin-2-ylamino]-4'-[4-chloro-6-di( $\beta$ -hydroxyethyl)amino-s-triazin-2-ylamino]-stilbene-2,2'-disulfonic acid  
 20. 2,8-bis[4-(4-sulfoanilino)-6-hydroxy-s-triazin-2-ylamino]-carbazole  
 21. 4,4'-bis(4,6-di( $\beta$ -hydroxyethylamino)-s-triazin-2-yl)benzi-dine-2,2'-disulfonic acid  
 22. 2-laurylaminio-4,6-di(4-sulfoanilino)-s-triazine  
 23. 4,4'-bis{4-[4'-(N',  
 24. 5-acetamido-2-(4-styryl-3-sulfo)phenyl-1,2,3-benzotriazole sodium salt  
 25. 2,7-diacetamido-3,6-disulfodibenzothiophene-5,5-dioxide sodium salt  
 26. 4-sulfo-o-terphenyl sodium salt (Lour. Organ. Chem., Vol. 14 (1949), pg. 163)  
 27. pyrene-3-(4-methoxy-3-sulfonyl)ketone sodium salt  
 28. 3,7-bis(4-methyl-2-methoxybenzamido)-2,8-disulfodibenzothiophene-5,5-dioxide sodium salt

As can be seen above, many of the sulfonated derivatives are employed in the form of their water-soluble salts, such as alkali metal (e.g., sodium, potassium, etc.) salts, or ammonium or amine (e.g., triethylamine, triethanolamine, pyridine, aniline, etc.) salts. By thus using these derivatives, they can be added to the emulsions in substantially neutral aqueous solutions without disturbing the pH of the emulsions.

In accordance with the practice of this invention, any reducing agent (i.e., a material capable of reducing silver halide) can be employed which coacts with the complex merocyanine dye and sulfonated polynuclear organic compound to further enhance the blue sensitivity of the silver halide emulsion. Particularly good results are employed with dihydroxy substituted reducing agents. Typical dihydroxy compounds which can be employed in the practice of this invention are selected from the group consisting of the benzenes, gamma-lactones, pyronimides, tetroximides, furans and pyrroles, which contain at least two hydroxyl groups.

Typical useful dihydroxy substituted compounds which can be utilized include hydroquinone, resorcinol, pyrocatechol, 3-methylpyrocatechol, toluhydroquinone, naphthalenediols, etc.;  $\gamma$ -lactones such as ascorbic acid, isoascorbic acid, etc.; 3-hydroxy tetroximides; 3,4,5-trihydroxy-5,6-dihydro-pyronimides; and amino hexose reductones wherein the moiety comprising the subject reductones can be represented by the following formula



wherein:  $R^1$  and  $R^2$  can be an alkyl radical, preferably having one to eight carbon atoms or together the necessary atoms to make a heterocyclic radical with the nitrogen atom, preferably having a five to six atom nucleus and including a second nitrogen atom or an oxygen atom such as morpholino, piperazino, pyrrolino, pyridino, pyrimidino, piperidino and the like.

The typical suitable tetroximides, pyronimides and amino hexose reductones are set out in Table B:

Table B

## 5-Phenyl-3-hydroxy tetroximide



- 5-(4-Carboxyphenyl)-3-hydroxy tetroximide,  
 5-(3,4-Dimethoxyphenyl)-3-hydroxy tetroximide,  
 5-(n-Butyl)-3-hydroxy tetroximide  
 5-(2-Furyl)-3-hydroxy tetroximide  
 5-(5-a-Furyl-3,4-dihydroxy-2-imino-2,5-dihydrofuran), and the like;  
 5,6-Diphenyl-3,4,5-trihydroxy-5,6-dihydro-pyronimide



- 15  
 20  
 25  
 30  
 35  
 40  
 45  
 50  
 55  
 60  
 65  
 70  
 75
- 5-(4-Carboxyphenyl)-3-hydroxy tetroximide,  
 5,6-Di-n-butyl-3,4,5-trihydroxy-5,6-dihydro-pyronimide,  
 5,6-Di-morpholino-3,4,5-trihydroxy-5,6-dihydro-pyronimide,  
 5,6-(2-Sulfophenyl)-3,4,5-trihydroxy-5,6-dihydro-pyronimide,  
 and the like;  
 Dimethylamino hexose reductone  
 Di-n-hexylamino  
 Di-n-butylamino hexose reductone Di-n-hexylamino hexose reductone  
 Morpholino hexose reduction  
 Piperazino hexose reductone  
 Pyrrolino hexose reductone  
 Piperidino hexose reductone and the like.

The tetroximides and pyronimides such as mentioned above may be prepared by the methods described in British Pat. No. 782,304, Swiss Pat. No. 322,985, and in Helv. Chim. Acta, 39, 1,780 (1956). The above, and still other 3-hydroxy tetroximides and 3,4,5-trihydroxy-5,6-dihydro-pyronimides that are suitable, are disclosed in Salminen, U.S. Pat. No. 3,330,655, issued July 11, 1967.

The amino hexose reductones of the invention are derived from sugars, especially D-glucose, although other six carbon or hexose reducing sugars such as D-galactose, D-mannose, D-fructose, L-sorbose or the like can be used. A typical method for preparing the subject reductones comprises heating in a reaction medium substantially free of water a hexose reducing sugar and an aliphatic or cyclic secondary amine in the presence of an acidic reductone-forming catalytic agent such as phosphoric acid, boric acid, acetic acid, succinic acid or the like. The removal of three molecules of water results during the formation of the subject amino hexose reductones. The mentioned reductones and other related suitable reductones and methods for preparing such are described in Hodges, U.S. Pat. No. 2,936,308.

According to the invention, one or more of the sulfonated organic compounds, one or more of the reducing agents and one or more of the complex merocyanine dyes of the invention are added singly or in combination to light-sensitive photographic silver halide emulsions to supersensitive the emulsions.

The invention is particularly directed to gelatino-silver-halide developing-out emulsions. However, the supersensitizing combinations can also be employed in silver halide emulsions in which the carrier or vehicle is a hydrophilic colloid other than gelatin, such as albumin, agar-agar, gum arabic, alginic acid, etc., or a hydrophilic resin such as polyvinyl alcohol, polyvinyl pyrrolidone, a cellulose ether, a partially hydrolyzed cellulose acetate, acrylamide polymers, etc., which has no deleterious effect upon the light-sensitive silver halide. The sulfonated organic compounds, and reducing agents and the dyes of Formula I above can be employed in the combination of the invention in various concentrations depending upon the particular emulsion, concentration of the silver halide, particular results desired, etc. The optimum concentration of an individual sensitizing dye can be determined in a manner well known to those skilled in the art by measuring the sensitivity of a series of test portions of the same emulsion, each portion containing a different concentration of the sensitizing dye. In general, the sulfonated organic compounds and reducing

agents in my invention have little or no sensitizing action by themselves alone in the emulsions employed. Ordinarily, the optimum or near optimum concentration of the complex merocyanine dyes herein is of the order of from 0.01 to 0.30 g. per mole of silver halide in the emulsion, and that of the sulfonated organic compound and reducing agents herein are of the order of from 0.50 to 4.0 g. and 1.0 to 8.0 g., respectively.

The methods of incorporating sensitizing dyes in silver halide emulsions are well known to those skilled in the art and these known techniques are employed in dispersing the dyes of the invention in the emulsions. In practicing my invention and the sensitizing dyes, the sulfonated organic compounds and the reducing agents can be directly dispersed in the emulsions, or they can first be dissolved in some convenient solvent, such as pyridine, methyl alcohol, acetone, etc. (or mixtures of such solvents), or diluted with water in some instances, and added to the emulsions in the form of these solutions. If desired, the components can be separately dissolved in a given solvent and added separately to the emulsion, or they can be dissolved in the same or different solvent and these solutions mixed together before addition is made to the silver halide emulsions. The dyes, sulfonated organic compounds and reducing agents of the invention are dispersed in the finished emulsions in such a manner as to be uniformly distributed throughout the emulsions prior to coating on a suitable support, such as paper, glass, cellulose ester film, polyvinyl resin film (e.g., polystyrene film, polyvinyl chloride film, etc.) polyester film, etc. The following procedure has been found quite satisfactory: Stock solutions of the sulfonated organic compounds, reducing agents and the dyes of Formula I above are prepared by separately dissolving these components in appropriate solvents as described above. Then, to the flowable silver halide emulsion, the desired amount of stock solution of one of the dyes is slowly added while stirring the emulsion. Stirring is continued until the dye is thoroughly incorporated in the emulsion. Then, the desired amount of stock solution of one of the sulfonated organic compounds is slowly added to the emulsion while stirring. Next, the desired amount of one of the reducing agents is added. Stirring is continued until the added materials are thoroughly incorporated in the emulsion. The supersensitized emulsions can then be coated on a suitable support and the coating allowed to dry. In some instances, it may be desirable to heat the supersensitized emulsion for a few minutes before coating onto the suitable support. The details of such coating techniques are well known to those skilled in the art. The foregoing procedure and proportions are to be regarded only as illustrative. Clearly, the invention is directed to any silver halide emulsion containing a supersensitizing combination of the invention, e.g., gelatino-silver chloride, -chlorobromide, -chloroiodide, -chlorobromoiodide, -bromoiodide, etc., emulsions.

Fine grain emulsions can also be employed herein. These may be prepared by precipitating photosensitive silver halide crystals, in an aqueous medium, in the presence of an acid substituted aryl mercaptan, e.g., thiosalicylic acid, dissolved in said medium. Gelatin or other suitable hydrophilic colloid is added and the emulsion obtained is chilled and set. The chilled emulsion is then shredded into small noodles and washed in running tap water. After washing, the emulsion is remelted, and the volume, pH and *Pag* are adjusted. A fine grain gelatino-silver bromoiodide emulsion prepared in the above manner and containing a dye combination of the invention is particularly useful for recording radiations in the region of the spectrum ranging about from 300 to 750 nm. in fine detail. Further details for preparing such fine-grain emulsions can be had by reference to copending application of Sutherlands, Ser. No. 622,034, filed March 10, 1967.

The emulsions of this invention can contain the chemical sensitizers, speed increasing compounds, plasticizers, hardeners and coating aids, and the silver halide may be dispersed in any of the binders, that are described and referred to in Graham et al. U.S. Pat. No. 3,046,129, issued July 24, 1962.

The following examples are included for further understanding of the invention.

#### EXAMPLES 1 to 7

5 These examples illustrate the supersensitization produced by various supersensitizing combinations of the invention containing a complex merocyanine dye defined by Formula I above in the region of the spectrum of wavelengths above about 510 nm. The testing procedure and the results are set forth in the following description and Table 1. The specified complex merocyanine dyes are identifiable by reference to above Table A, while the specific sulfonated organic compounds and reducing agents are named in the footnotes to the following table of these examples.

10 To different portions of the same batch of melted gelatino-silver bromoiodide emulsion, containing 0.77 mole percent iodide, of the type described by Trivelli and Smith, Phot. Journal, 79, 330 (1939), are added the individual complex merocyanine dyes, sulfonated organic compounds and reducing agents in the proportions given in Table 1 hereinafter. In each case, after being digested at about 40° C. for 5 minutes, the emulsion is coated at a coverage of 432 mg. silver per square foot on a cellulose acetate film support. A sample of each coating is exposed on an Eastman 1B Sensitometer to light from a tungsten source modulated by a step-wedge and Kodak Wratten No. 16 filter and processed for 3 minutes at 20° C. in Kodak developer D-19 which has the following composition:

|    |                                |         |
|----|--------------------------------|---------|
| 30 | N-methyl-p-aminophenol sulfate | 2.0 g.  |
|    | Hydroquinone                   | 8.0 g.  |
|    | Sodium sulfite (desiccated)    | 90.0 g. |
|    | Sodium carbonate (monohydrate) | 52.5 g. |
|    | Potassium bromide              | 5.0 g.  |
|    | Water to make                  | 1.0 g.  |

35 and then fixed in a conventional sodium thiosulfate fixing bath, washed and dried. Densitometric measurements are then made of the developed images of each coating. The relative speed values are determined by the exposure necessary to produce a density of 0.3 above fog, an arbitrary relative speed of 100, or more as indicated, being chosen for the control containing no dye. The results are listed in the following table together with the values for gamma and fog.

40 TABLE 1  
Supersensitization of complex merocyanine dyes

| Ex. No. | Dye No. and conc. (g./mole silver) | Addendum and conc. (g./mole silver) | Relative minus blue speed (#16 wratten) filter |      |     |
|---------|------------------------------------|-------------------------------------|------------------------------------------------|------|-----|
|         |                                    |                                     | $\gamma$                                       | Fog  |     |
| 50      | 1:                                 |                                     |                                                |      |     |
|         | (a) I .03                          | None                                | 100                                            | 1.62 | .06 |
|         | (b) I .03                          | A .15                               | 316                                            | 1.53 | .06 |
|         | (c) I .03                          | X .75                               | 219                                            | 1.35 | .04 |
|         | (d) I .03                          | A+X 1.5+.75                         | 417                                            | 1.58 | .05 |
| 55      | 2:                                 |                                     |                                                |      |     |
|         | (a) II .03                         | None                                | 100                                            | 1.66 | .05 |
|         | (b) II .03                         | A .15                               | 302                                            | 1.83 | .08 |
|         | (c) II .03                         | X .75                               | 182                                            | 1.32 | .04 |
|         | (d) II .03                         | A+X 1.5+.75                         | 575                                            | 1.60 | .06 |
| 60      | 3:                                 |                                     |                                                |      |     |
|         | (a) III .03                        | None                                | 151                                            | 1.46 | .06 |
|         | (b) III .03                        | A .15                               | 106                                            | 1.15 | .08 |
|         | (c) III .03                        | X .75                               | 331                                            | 1.32 | .06 |
|         | (d) III .03                        | A+X 1.5+.75                         | 417                                            | 1.27 | .06 |
| 65      | 4:                                 |                                     |                                                |      |     |
|         | (a) IV .03                         | None                                | 479                                            | 1.59 | .05 |
|         | (b) IV .03                         | B .15                               | 501                                            | 1.52 | .06 |
|         | (c) IV .03                         | X .75                               | 601                                            | 1.50 | .05 |
|         | (d) IV .03                         | B+X 1.5+.75                         | 726                                            | 1.60 | .06 |
| 70      | 5:                                 |                                     |                                                |      |     |
|         | (a) V .03                          | None                                | 87                                             | 2.14 | .06 |
|         | (b) V .03                          | A .15                               | 132                                            | 1.92 | .06 |
|         | (c) V .03                          | X .75                               | 174                                            | 1.92 | .04 |
|         | (d) V .03                          | A+X 1.5+.75                         | 151                                            | 1.60 | .04 |
| 75      | 6:                                 |                                     |                                                |      |     |
|         | (a) VI .03                         | None                                | 35                                             | 1.42 | .04 |
|         | (b) VI .03                         | B .15                               | 38                                             | 1.57 | .04 |
|         | (c) VI .03                         | X .75                               | 80                                             | 1.18 | .06 |
|         | (d) VI .03                         | B+X 1.5+.75                         | 91                                             | 1.42 | .06 |
|         | (e) VII .03                        | C .15                               | 178                                            | 1.74 | .04 |
|         | (f) VII .03                        | X .75                               | 331                                            | 1.55 | .04 |
|         | (g) VII .03                        | A .15                               | 324                                            | 1.78 | .06 |
|         | (h) VII .03                        | A+X 1.5+.75                         | 537                                            | 1.73 | .04 |
|         | (i) VII .03                        | C .15                               | 339                                            | 1.64 | .04 |
|         | (j) VII .03                        | C+X 1.5+.75                         | 490                                            | 1.74 | .05 |

|          |     |     |          |         |     |      |     |
|----------|-----|-----|----------|---------|-----|------|-----|
| (g)..... | VII | .03 | B.....   | 1.5     | 309 | 1.87 | .06 |
| (h)..... | VII | .03 | B+X..... | 1.5+.75 | 513 | 1.71 | .05 |
| (i)..... | VII | .03 | D.....   | 1.5     | 282 | 1.85 | .05 |
| (j)..... | VII | .03 | D+X..... | 1.5+.75 | 436 | 1.75 | .05 |
| (k)..... | VII | .03 | E.....   | 1.5     | 380 | 1.80 | .06 |
| (l)..... | VII | .03 | E+X..... | 1.5+.75 | 501 | 1.70 | .04 |
| (m)..... | VII | .03 | F.....   | 1.5     | 276 | 1.60 | .08 |
| (n)..... | VII | .03 | F+X..... | 1.5+.75 | 398 | 1.64 | .06 |

## Addendum.

X = Calcofluor White MR is a sulfonated triazinyl stilbene e.g., a bis(s-triazin-2-ylamino)stilbene-2,2'-disulfonic acid (sodium salt).  
 A = Ascorbic acid.  
 B = Piperadino hexose reductone.  
 C = d-Isoascorbic acid.  
 D = Hydroquinone.  
 E = 5,6-di-phenyl-3,4,5-trihydroxy-5,6-dihydro pyronimide.  
 F = 5- $\alpha$ -furyl-3,4-di-hydroxy-2-imino-2,5-di-hydrofuran.

Referring to above Table 1, it will be seen that in each example the supersensitizing combinations of the invention comprising dye + sulfonated organic compound + reducing agent produces markedly increased minus blue speed in the light-sensitive emulsion over that produced by the dye plus sulfonated organic compound, and that the supersensitizing effect of the sulfonated organic compound and the reducing agent is clearly additive as shown in all of the examples and more particularly with the comparisons in Example 7.

## EXAMPLES 8-12

These examples illustrate that the inclusion of a reducing agent of the invention into the supersensitizing combinations herein decreases the desensitization of the complex merocyanine dyes of the invention. The testing procedure is exactly the same as that described for above Examples 1 to 7, except that the exposures of the samples are made through Wratten Filter No. 35 + Wratten Filter No. 38A + Chance Glass Filter (which combination transmits only light in the blue region of the spectrum), thereby giving relative blue speeds for each of the examples. The results of these tests are set forth in the following Table 2.

TABLE 2  
Decrease in desensitization of complex merocyanine dyes by addition of reducing agent

| Ex. No.  | Dye No. and conc. (g./mole silver) | Addendum and conc. (g./mole silver) | Relative blue speed #35+38A Wratten filters plus Chance glass fil. | $\gamma$ | Fog |
|----------|------------------------------------|-------------------------------------|--------------------------------------------------------------------|----------|-----|
| 8:       |                                    |                                     |                                                                    |          |     |
| (a)..... | I                                  | .03 None.....                       | 27.5 1.36                                                          | .06      |     |
| (b)..... | I                                  | .03 A..... 1.5                      | 60 1.34                                                            | .06      |     |
| (c)..... | I                                  | .03 X..... 0.75                     | 36 1.20                                                            | .04      |     |
| (d)..... | I                                  | .03 A+X..... 1.5+.75                | 76 1.33                                                            | .06      |     |
| 9:       |                                    |                                     |                                                                    |          |     |
| (a)..... | II                                 | .03 None.....                       | 19 1.36                                                            | .05      |     |
| (b)..... | II                                 | .03 A..... 1.5                      | 40 1.50                                                            | .08      |     |
| (c)..... | II                                 | .03 X..... 0.75                     | 18 1.02                                                            | .05      |     |
| (d)..... | II                                 | .03 A+X..... 1.5+.75                | 53 1.46                                                            | .06      |     |
| 10:      |                                    |                                     |                                                                    |          |     |
| (a)..... | V                                  | .03 None.....                       | 115 1.63                                                           | .04      |     |
| (b)..... | V                                  | .03 A..... 1.5                      | 151 1.41                                                           | .06      |     |
| (c)..... | V                                  | .03 X..... 0.75                     | 123 1.53                                                           | .04      |     |
| (d)..... | V                                  | .03 A+X..... 1.5+.75                | 138 1.35                                                           | .05      |     |
| 11:      |                                    |                                     |                                                                    |          |     |
| (a)..... | VI                                 | .03 None.....                       | 78 1.35                                                            | .04      |     |
| (b)..... | VI                                 | .03 B..... 1.5                      | 87 1.43                                                            | .05      |     |
| (c)..... | VI                                 | .03 X..... 0.75                     | 67 1.15                                                            | .05      |     |
| (d)..... | VI                                 | .03 B+X..... 1.5+.75                | 83 1.25                                                            | .06      |     |
| 12:      |                                    |                                     |                                                                    |          |     |
| (a)..... | VII                                | .03 None.....                       | 58 1.46                                                            | .06      |     |
| (b)..... | VII                                | .03 X..... 0.75                     | 54 1.34                                                            | .03      |     |
| (c)..... | VII                                | .03 A..... 1.5                      | 54 1.44                                                            | .08      |     |
| (d)..... | VII                                | .03 A+X..... 1.5+.75                | 95 1.48                                                            | .05      |     |
| (e)..... | VII                                | .03 C..... 1.5                      | 95 1.52                                                            | .07      |     |
| (f)..... | VII                                | .03 C+X..... 1.5+.75                | 105 1.45                                                           | .06      |     |
| (g)..... | VII                                | .03 B..... 1.5                      | 87 1.50                                                            | .06      |     |
| (h)..... | VII                                | .03 B+X..... 1.5+.75                | 95 1.40                                                            | .04      |     |
| (i)..... | VII                                | .03 D..... 1.5                      | 76 1.54                                                            | .05      |     |
| (j)..... | VII                                | .03 D+X..... 1.5+.75                | 76 1.56                                                            | .04      |     |
| (k)..... | VII                                | .03 E..... 1.5                      | 69 1.52                                                            | .06      |     |
| (l)..... | VII                                | .03 E+X..... 1.5+.75                | 73 1.46                                                            | .04      |     |
| (m)..... | VII                                | .03 F..... 1.5                      | 55 1.40                                                            | .09      |     |
| (n)..... | VII                                | .03 F+X..... 1.5+.75                | 73 1.44                                                            | .04      |     |

## Addendum:

X = Calcofluor White MR.  
 A = Ascorbic acid.  
 B = Piperadino hexose reductone.  
 C = d-Isoascorbic acid.  
 D = Hydroquinone.  
 E = 5,6-di-phenyl-3,4,5-trihydroxy-5,6-dihydro pyronimide.  
 F = 5- $\alpha$ -furyl-3,4-di-hydroxy-2-imino-2,5-di-hydrofuran.

It will be noted from above Table 2 that the addition of the specified reducing agents produce a substantial improvement in the relative blue speed in each of the examples which contain just dye and sulfonated organic compound.

5

## EXAMPLES 13-15

These examples show that the addition of the reducing agents of the invention to dicarbocyanine dyes with the sulfonated organic compounds herein do not give any superadditivity over the dye with the sulfonated organic compound along (A of Table 3), or show any significant decrease in desensitization (B of Table 3). The comparison dicarbocyanine dyes are identifiable from the footnotes following Table 3. The testing procedure is exactly the same as that described for above Examples 8 to 12. The results of these tests are listed in Table 3 immediately below.

TABLE 3

A. Decrease in sensitization ratio of dicarbocyanine dyes with addition of reducing agent to dye and Calcofluor White MR (dye Nos. VIII and IX)

| Ex. No.  | Dye No. and conc. (g./mole silver) | Addendum and conc. (g./mole silver) | Relative blue speed (#35+38A Wratten filter plus Chance glass fil.) | $\gamma$ | Fog |
|----------|------------------------------------|-------------------------------------|---------------------------------------------------------------------|----------|-----|
| 13:      |                                    |                                     |                                                                     |          |     |
| (a)..... | VIII                               | .03 None.....                       | 40 1.22                                                             | .04      |     |
| (b)..... | VIII                               | .03 A..... 1.5                      | 44 1.03                                                             | .22      |     |
| (c)..... | VIII                               | .03 X..... 0.75                     | 427 1.45                                                            | .05      |     |
| (d)..... | VIII                               | .03 A+X..... 1.5+.75                | 276 1.20                                                            | .08      |     |
| 14:      |                                    |                                     |                                                                     |          |     |
| (a)..... | IX                                 | .03 None.....                       | 58 1.00                                                             | .04      |     |
| (b)..... | IX                                 | .03 A..... 1.5                      | 73 1.12                                                             | .10      |     |
| (c)..... | IX                                 | .03 X..... 0.75                     | 295 1.46                                                            | .05      |     |
| (d)..... | IX                                 | .03 A+X..... 1.5+.75                | 151 1.18                                                            | .06      |     |

B. Effect on desensitization of dicarbocyanine dyes by addition of reducing agent

|          |      |                      |         |     |  |
|----------|------|----------------------|---------|-----|--|
| 14:      | VIII | .03 None.....        | 100 1.2 | .03 |  |
| (b)..... | VIII | .03 A..... 1.5       | 91 0.95 | .30 |  |
| (c)..... | VIII | .03 X..... 0.75      | 94 0.50 | .12 |  |
| (d)..... | VIII | .03 A+X..... 1.5+.75 | 91 1.03 | .12 |  |
| 15:      |      |                      |         |     |  |
| (a)..... | IX   | .03 None.....        | 82 1.23 | .03 |  |
| (b)..... | IX   | .03 A..... 1.5       | 83 1.06 | .14 |  |
| (c)..... | IX   | .03 A+X..... 0.75    | 91 1.16 | .04 |  |
| (d)..... | IX   | .03 A+X..... 1.5+.75 | 91 0.07 | .07 |  |

Addendum: A and X are as defined in above Examples 1 to 8; Dye No. 45: 3,3'-diethyl thiadicarbocyanine iodide; Dye No. IX: 3,3'-diethyl sebenadicarbocyanine iodide.

By reference to above Table 3, it will be clearly evident that dicarbocyanine dyes do not produce the advantageous supersensitization results found with the complex merocyanine dye combinations of the invention.

## EXAMPLES 16-17

These examples indicate that simple merocyanine dyes are not supersensitized by either the reducing agent, by Calcofluor White MR or by the combination of these two compounds (A of Table 4), and show only slight decrease in desensitization (B of Table 4). The simple merocyanine dye in these examples is identifiable from the footnote to the Table.

The testing procedure is exactly the same as described in the foregoing examples for both A and B sections of the Table, except that the exposures for A are made through Wratten Filters No. 35 + No. 38A + Chance Glass Filter (for relative minus blue speed, etc.). The test values appear in the following Table 4.

TABLE 4

A. Decrease in sensitization ratio of a simple merocyanine dye with addition of reducing agent to the dye with Calcofluor White MR (dye No. X)

| Ex. No.  | Dye No. and conc. (g./mole silver) | Addendum and conc. (g. mole silver) | Relative minus blue speed (#18 filter) | $\gamma$ | Fog |
|----------|------------------------------------|-------------------------------------|----------------------------------------|----------|-----|
| 16:      |                                    |                                     |                                        |          |     |
| (a)..... | X                                  | .08 None.....                       | 457 1.50                               | .06      |     |
| (b)..... | X                                  | .08 A..... 4.0                      | 457 1.40                               | .12      |     |
| (c)..... | X                                  | .08 X..... 2.0                      | 302 0.94                               | .06      |     |
| (d)..... | X                                  | .08 A+X..... 4+2                    | 347 1.37                               | .10      |     |

**B. Effect on desensitization of a simple merocyanine dye by addition of a reducing agent (dye No. X)**

|     |          |   |     |           |     |      |     |
|-----|----------|---|-----|-----------|-----|------|-----|
| 17: | (a)..... | X | .08 | None..... | *82 | 1.15 | .05 |
|     | (b)..... | X | .08 | A.....    | 105 | 0.70 | .22 |
|     | (c)..... | X | .08 | X.....    | 95  | 1.40 | .05 |
|     | (d)..... | X | .08 | A+X.....  | 132 | 1.15 | .17 |

\* Relative blue speed (Wratten filters #35 plus #38A plus Chance glass filter).

Addendum: A and X are as defined in above Examples 1 to 8. Dye No. X: 5-[(3-ethyl-2-benzothiazolidene)ethylidene]-3-ethylrhodanine.

Referring to above Table 4, it will be seen that simple merocyanine dyes also do not produce the advantageous supersensitizing results of the complex merocyanine combinations of this invention.

It will be understood that any other complex merocyanine dye defined by Formula I above can be substituted in the preceding examples of the invention to give generally similar advantageous supersensitizing results for light-sensitive photographic silver halide emulsions. Also, the sulfonated organic compounds and reducing agents in the supersensitizing combinations of the examples can be substituted with any other of those previously mentioned as being suitable with similar advantageous supersensitizing results for such emulsions.

Although the invention has been described in considerable detail with particular reference to certain preferred embodiments thereof, it will be understood that variations and modifications can be effected within the spirit and scope of the invention.

I claim:

1. A photographic silver halide emulsion sensitized with a combination comprising (1) a complex merocyanine dye having three five- to six-membered nitrogen containing heterocyclic nuclei joined at a carbon atom thereof by a linkage selected from the group consisting of a double bond and a methine linkage, one terminal nucleus of said dye being a basic heterocyclic nucleus of the type used in cyanine dyes, and the other two nuclei of said dye being acidic ketomethylene heterocyclic nuclei of the type used in merocyanine dyes, said dye having the amidic chromophoric system; (2) a sulfonated polynuclear aromatic organic super-sensitizer; and, (3) sufficient amount of a silver halide reducing agent to effectively increase the blue speed of the emulsion.

2. A photographic silver halide emulsion spectrally sensitized with (1) a complex merocyanine dye represented by the following formula:



wherein  $n$  represents a positive integer of from 1 to 2;  $m$  and  $p$  each represents a positive integer of from 1 to 3; L represents a methine linkage;  $R_1$  represents a member selected from the group consisting of an alkyl group and an aryl group; A represents a member selected from the group consisting of an atom of sulfur and the group  $=N-R_3$ ;  $R_2$  and  $R_3$  each represents a member selected from the group consisting of an alkyl group containing from one to four carbon atoms and an aryl group; Z represents the nonmetallic atoms necessary to complete a heterocyclic nucleus of the type used in cyanine dyes containing from five to six atoms in the heterocyclic ring; and Q represents the nonmetallic atoms necessary to complete a heterocyclic nucleus selected from the group consisting of a 2-pyrazolin-5-one nucleus; a 2-thiobarbituric acid nucleus; and, a rhodanine nucleus; (2) a water-soluble sulfonated organic compound represented by the following formula:

wherein B<sub>1</sub> represents a 1,3,5-triazin-6-ylamino group, B<sub>2</sub> represents an aromatic group, and M represents a member selected from the group consisting of a hydrogen atom and an alkali metal atom; and (3) a dihydroxy substituted reducing agent selected from the group consisting of the benzenes, gamma lactones, tetroneimides, pyronimides, furans and pyrroles which contain at least two hydroxyl groups.

10 3. A photographic silver halide emulsion sensitized with a supersensitizing combination comprising (1) a complex merocyanine dye represented by the following formula:



wherein  $n$  represents a positive integer of from 1 to 2;  $m$  and  $p$  each represents a positive integer of from 1 to 3;  $L$  represents a methine linkage;  $R_1$  represents a member selected from the group consisting of an alkyl group and an aryl group;  $A$  represents a member selected from the group consisting of an atom of sulfur and the group  $=N-R_3$ ;  $R_2$  and  $R_3$  each represents a member selected from the group consisting of an alkyl group containing from one to four carbon atoms and an aryl group;  $Z$  represents the nonmetallic atoms necessary to complete a heterocyclic nucleus of the type used in cyanine dyes containing from five to six atoms in the heterocyclic ring; and  $Q$  represents the nonmetallic atoms necessary to complete a heterocyclic nucleus selected from the group consisting of a 2-pyrazolin-5-one nucleus; a 2-thio-barbituric acid nucleus; and a rhodanine nucleus; (2) a water-soluble sulfonated organic compound represented by the following formula:



wherein  $B_1$  represents a 1,3,5-triazin-6-ylamino group,  $B_2$  represents an aromatic group, and  $M$  represents a member selected from the group consisting of a hydrogen atom and an alkali metal atom; and (3) an organic reducing agent containing at least two hydroxyl group substituents selected from the class consisting of a dihydroxyarylene; a  $\lambda$ -lactone; a 3-hydroxy tetronamide; a 3,4,5-trihydroxy-5,6-dihydropyronimide; and, an amino hexose reductone wherein the amino moiety of said reductone has the formula:



wherein R<sup>1</sup> and R<sup>2</sup> are selected from the group consisting of  
60 alkyl radicals and together with the nitrogen atom the necessary  
atoms to form a nitrogen-containing heterocyclic radical.

4. A photographic silver halide emulsion spectrally sensitized with a complex merocyanine dye selected from the group consisting of: 1-ethyl-4-[(3-ethyl-2-benzothiazolinylidene)-ethylidene]-2-[(3-ethyl-4-oxo-2-thioxo-5-thiazolidinylidene)-ethylidene]-3-phenyl-5-imidazolidinone; 1,3-diethyl-5-[(1-ethylnaphtho[1,2-d]thiazolin-2-ylidene)ethylidene]-2-[(3-ethyl-4-oxo-2-thioxo-5-thiazolidinylidene)ethylidene]lg0-4-imidazolidinone; 3-ethyl-2-[(1-ethylhexahydro-4,6-dioxo-2-thioxo-5-pyrimidinylidene)-ethylidene]-1-phenyl-5-[(1,3,3-trimethyl-2-indolinylidene)ethylidene]-4-imidazolidinone; 1,3-diethyl-5-[(3-ethyl-2-benzothiazolinylidene)ethylidene]-2-[(3-methyl-5-oxo-1-phenyl-2-pyrazolin-4-ylidene)ethylidene]-4-



o-5-thiazolidinylidene)ethylidene]-4-thiazolidinone; 3-ethyl-5-[(1-ethylnaphtho[1,2-d]thiazolin-2-ylidene)ethylidene]-2-[(3-ethyl-4-oxo-2-thioxo-5-thiazolidinylidene)ethylidene]-1-phenyl-4-imidazolidinone; said emulsion being supersensitized with a sulfonated triazinylstilbene and a reducing agent selected from the group consisting of a dihydroxy substituted benzene; ascorbic acid; isoascorbic acid; 5- $\alpha$ -furyl-3,4-dihydroxy-2-imino-2,5-dihydrofuran; 5,6-diphenyl-3,4,5-trihydroxy-5,6-dihydro-pyronimide; and piperidino hexose reductone.

5. A photographic silver halide emulsion supersensitized with the combination of 1-ethyl-4-[(3-ethyl-2-benzothiazolinylidene)ethylidene]-2-[(3-ethyl-4-oxo-2-thioxo-5-thiazolidinylidene)ethylidene]-3-phenyl-5-imidazolidinone; ascorbic acid; and a bis(s-triazin-2-ylamino)stilbene-2,2'-disulfonic acid, sodium salt.

6. A photographic silver halide emulsion supersensitized with the combination of 1,3-diethyl-5-[(1-ethylnaphtho[1,2-d]thiazolin-2-ylidene)ethylidene]-2-[(3-ethyl-4-oxo-2-thioxo-5-thiazolidinylidene)ethylidene]-4-imidazolidinone; ascorbic acid; and, a bis(s-triazin-2-ylamino)stilbene-2,2'-disulfonic acid, sodium salt.

7. A photographic silver halide emulsion supersensitized with the combination of 3-ethyl-5-[(1-ethylnaphtho[1,2-d]thiazolin-2-ylidene)ethylidene]-2-[(3-ethyl-4-oxo-2-thioxo-5-thiazolidinylidene)ethylidene]-4-0-1-phenyl-4-imidazolidinone; ascorbic acid; and, a bis(s-triazin-2-ylamino)stilbene-2,2'-disulfonic acid, sodium salt.

8. A photographic silver halide emulsion supersensitized with the combination of 1,3-diethyl-5-[(3-ethyl-2-benzothiazolinylidene)ethylidene]-2-[(3-methyl-5-oxo-1-phenyl-2-pyrazolin-4-ylidene)ethylidene]-4-imidazolidinone; piperadino hexose reductone; and, a bis(s-triazin-2-ylamino)stilbene-2,2'-disulfonic acid, sodium salt.

9. A photographic silver halide emulsion supersensitized with the combination of 3-ethyl-5-[(1-ethylnaphtho[1,2-d]thiazolin-2-ylidene)ethylidene]-2-[(3-ethyl-4-oxo-2-thioxo-5-thiazolidinylidene)ethylidene]-4-0-1-phenyl-4-imidazolidinone; 5,6-di-phenyl-3,4,5-trihydroxy-5,6-dihydro pyronimide; and, a bis(s-triazin-2-ylamino)stilbene-2,2'-disulfonic acid, sodium salt.

15 20 \* \* \* \* \*

UNITED STATES PATENT OFFICE  
CERTIFICATE OF CORRECTIONPatent No. 3,649,289Dated March 14, 1972Inventor(s) Gary L. Hiller

It is certified that error appears in the above-identified patent and that said Letters Patent are hereby corrected as shown below:

Column 1, line 56, "a" should read ---the---.

Column 2, line 35, that part of formula reading "naphto" should read ---naphtho---.

Column 2, line 40, "5methyloxazole" should read --- 5-methyl-oxazole ---.

Column 2, line 51, "5chlorobenzoselenazole" should read --- 5-chlorobenzoselenazole ---.

Column 3, line 16, that part of formula reading "31(4" should read --- 3-(4- ---.

Column 3, line 19, "3-phenylrhodanine" should read --- 3-phenylrhodanine ---.

Column 3, line 38, that part of formula reading "ethyldene<sup>7</sup>" should read --- ethyldene<sup>7-1</sup> ---.

Column 3, line 56, that part of formula reading "ethyldene<sup>7</sup>" should read --- ethyldene<sup>7-1</sup> ---.

Column 4, line 37, "(2.0(ml.))" should read ---(2.0 ml.)---.

Column 4, line 63, "pyradinium" should read ---pyridinium---

Column 7, line 5, that part of formula reading "4-L-phenoxy" should read --- 4-L-phenoxy ---.

Column 8, line 23, "Di-n-hexylamino" should be deleted.

Column 8, lines 24-25, "Di-n-hexylamino hexose reductone" sh  
be on a separate line and not a continuation of the line in  
which it has been printed.

PO-1050  
(5/69)UNITED STATES PATENT OFFICE  
CERTIFICATE OF CORRECTIONPatent No. 3,649,289Dated March 14, 1972Inventor(s) Gary L. Hiller

It is certified that error appears in the above-identified patent and that said Letters Patent are hereby corrected as shown below:

Column 8, line 26, "reduction" should read ---reductone---.

Column 8, line 55, "supersensitive" should read ---super-sensitize---.

Column 8, line 61, before "albumin" ---, for example, --- should be inserted.

Column 9, line 12, before "the sensitizing" "and" should be deleted.

Column 9, lines 32-33, "inappropriate" should read ---in appropriate---.

Column 10, line 34, "1.0 g." should read ---1.0 liter---.

Column 11, line 8, that part of formula reading "2,2'-disulfon should read ---2,2'-disulfonic---.

Column 11, line 12, "Hydropuinone" should read ---hydroquinone---.

Column 12, line 12, "along" should read ---alone---.

Column 12, line 43, "A+X" should read ---X---.

Column 13, line 8, "4+5" should read ---4+2---.

Column 13, line 48, "sliver" should read ---silver---.

Column 14, line 68, that part of formula reading "thioxo-5-thioxo-5'" should read ---thioxo-5- ---.

Column 14, line 69, that part of formula reading "g0-4" should read --- -4 ---.

PO-1050  
(5/69)

UNITED STATES PATENT OFFICE  
CERTIFICATE OF CORRECTION

Patent No. 3,649,289

Dated March 14, 1972

Inventor(s) Gary L. Hiller

It is certified that error appears in the above-identified patent  
and that said Letters Patent are hereby corrected as shown below:

Column 15, line 9, that part of formula reading  
"5,6dihydro" should read ---5,6-dihydro---.

Column 16, line 4, that part of formula reading "g0-1"  
should read --- -1 ---.

Column 16, line 13, "slat" should read ---salt---.

Column 16, line 17, that part of formula reading "g0-1"  
should read --- -1 ---.

Column 16, line 20, "slat" should read ---salt---.

Signed and sealed this 12th day of September 1972.

(SEAL)

Attest:

EDWARD M. FLETCHER, JR.  
Attesting Officer

ROBERT GOTTSCHALK  
Commissioner of Patent